# EUROPEAN PATENT SPECIFICATION

(11) **EP 1 591 582 B1**
(45) Date of publication and mention of the grant of the patent: **28.10.2009**
(21) Application number: 05103211.8
(22) Date of filing: 21.04.2005
(51) Int. Cl.: D06Q 1/02, D06L 3/02, D06P 5/00, D06P 5/15

(54) **Printing process on raw textile materials**
Druckverfahren auf Rohtextilmaterialien
Procédé d'impression sur des textiles bruts

(30) Priority: 26.04.2004 IT FI20040098
(43) Date of publication of application: 02.11.2005
(73) Proprietor: Stamperia Altair S.r.l., 59100 Prato (IT)
(72) Inventor: Paolo, Lenzi, 59100, Prato (IT)
(74) Representative: Bardini, Marco Luigi

(56) References cited:
- EP-A- 0 449 797
- GB-A- 793 733
- JP-A- 52 148 288
- JP-A- 54 088 376
- US-A- 4 247 295

## Description

The present invention concerns the field of textile production. More specifically, it concerns a new process for obtaining surface designs through printing on raw textile materials.

Textile printing, in general terms, consists of applying printing pastes - containing dyes or pigments - to manufactured textile products. This step is followed by one or more stabilization steps, comprising physical and/or chemical treatments having the purpose of stably and locally fixing the dying substances. The textile print can be classified based upon the system of application - i.e. the system with which the dying substances are applied - and the processing techniques. As for the classification based upon the system of application, the following fundamental types are to be mentioned:
a) direct or application printing;
b) corrosion printing;
c) resist printing;
d) special prints (transfer or thermal transfer printing, Vigoureux printing, dévoré printing, flock printing, relief printing, printing with foil-coverage effects).

Based upon the processing techniques, the following division can then be made: screen printing (with manual, semi-automatic or automatic systems), hollow cylinder (rotary) printing, cylinder or roller printing.

All of the aforementioned treatments are well known to the average man skilled in the art, and will not be described in detail. However, in order to place the present description in the proper context, it is useful to sum up the characteristics of the three main systems of application.

Direct or application printing is the simplest process. It consists of a direct reproduction of patterns, in one or more colors, on white or lightly colored fabrics. A characteristic of application printing is the reproduction of the pattern on just one side of the textile product. In general, the processing sequence comprises the following steps: I.printing; II.drying; III.fixation/steaming; IV.washing; V.drying. In case of printing with pigments the sequence comprises the first three steps only.

Corrosion printing is carried out on fabrics dyed beforehand with corrodible dyes, i.e. dyes that can be degraded or discolored by a reducing etching during the steaming step. The corrosion can create a completely white pattern when, in addition to the corroding agent, white pigments (e.g. titanium dioxide) and optical bleaches are used. Very refined and sophisticated pattern motifs, and a rather low print coverage can be obtained. These are the two main reasons that lead to the choice of the corrosion printing process. With this process, effects of "illumination" are obtained with very intricate designs that cannot be made by direct printing.

Resist printing has the fundamental characteristic of preventing the fixation - in the printed area - of the base dye applied before or after printing. The result is similar to the one obtained by corrosion printing, but resist printing has the advantage of being more cost-effective, when it can replace corrosion. In general, resist printing can be obtained through physical resistance, i.e. application of printing pastes that prevent contact between the fiber and the dye in the subsequent dyeing step (for example batik print), or else chemical resistance, i.e. application of printing pastes containing chemical products that prevent the development of the dye in the printed areas.

A known printing method according to the preamble of annexed claim 1 is described in US4247295. In said method, a printing method is disclosed wherein a printing paste comprises an indigo dyestuff remover for discharge printing of textiles dyed with indigo blue. The printing paste may also contain a conventional bleaching agent when the print is to be made white.

The applicant has now identified a printing process that does not fit into any of the aforementioned known types and that, thanks to novel operating steps, allows a particularly good result to be accomplished in terms of quality and appearance of the textile product obtained, with advantages in terms of simplicity and speed of production, and consequently a favorable impact upon the relative costs.

Such a result is achieved, according to the present invention, with a printing process that can be used on a raw textile substrate made of natural and/or artificial cellulose fibers, alone or in combination with raw and/or dyed yarns of different composition, the essential features of which are defined by attached claim 1.

In practice, a localized bleaching according to a certain pattern is carried out through the application of the oxidative agent, namely simple hydrogen peroxide contained in a paste for printing with special characteristics and preparation. The paste is
characterized in particular by a very high concentration of hydrogen peroxide and of a strong base (notably sodium hydroxide), a concentration that can vary according to the heaviness and type of raw fabric to be treated, as well as to the degree of whitening that one wishes to obtain, but which is in any case around ten times the maximum normally used in conventional oxidative bleaching processes of cellulose fabrics. The pattern effect is therefore linked to the oxidative degradation of the natural pigments present in the cellulose fibers, caused by the oxidative agent in the aforementioned processing conditions that shall be described in greater detail later on.

The development of the oxidative action is thus improved during a subsequent drying step with hot air, which preferably takes place in a drying chamber with moderate ventilation at a temperature of between about 65° and 110°C. The drying time can vary between about 1 and 3 minutes and at the end the fabric is left to rest (folded in laps) for about 12 hours.

The printing paste can be applied, both on fabrics and on manufactured garments, by means of any one of the conventional processing techniques, i.e. with screen printing (with manual, semi-automatic or automatic systems), hollow cylinder (rotary) printing, cylinder printing or roller printing. The result is basically that of a textile substrate having the base color typical of raw manufactured products made of cellulose fibers - i.e. variable from light yellow up to dark grey - in which various types of printed patterns (geometric, flowery, fancy patterns etc.), are formed in lighter color than the base color, with variable penetration effect so that the print is visible only on the front of the fabric or else visible both on the front and on the reverse (two-sided effect) .

A result in some ways comparable to that obtained according to the invention could be achieved with the methods of the prior art only at the expense of rather long and complex operating steps, and/or in any case unable to ensure an outcome of the same quality. For instance, with a corrosion printing treatment, it would be necessary to preliminarily clean and bleach the raw manufactured textile products, to subsequently dye said products in the characteristic tones of natural cellulose fibers by using corrodible dyes, and finally to carry out the pattern effect with the actual corrosion print, this last step, moreover, being intrinsically lengthy and expensive. As an alternative, by carrying out pigment printing on raw substrates, the printing pattern could be obtained via a direct application of printing pastes with white pigments (e.g. titanium dioxide). In this case, however, the fabric shall have the typical characteristics of materials printed with pigments, first of all a fabric that is remarkably stiffer and harsher, and a print effect that is visible exclusively on the right side of the fabric.

Other characteristics and advantages of the printing process for obtaining surface designs on raw textile materials, and of the textile products thus obtained according to the present invention shall become clearer from the following description of an embodiment thereof, given purely as a non-limiting example.

According to the invention, the process can be used on yarns, fabrics and manufactured garments made of yarns of raw linen, raw cotton and whatever other cellulose fiber of natural and artificial origin; or else, it can be used on fabrics and manufactured garments made of raw yarns with a composition 100% of natural and artificial cellulose fibers, along with yarns with a different fiber composition, these being raw and/or dyed. The textile products mentioned above, in order to eradicate any possible traces of heavy metals that may sometimes be present (for example iron salts and/or oxides), are preferably pretreated with the conventional bating and complexation processes normally used in dyeing pretreatment cycles of cellulose textile materials. As an example, the following is a recipe for acid bating treatment.

**Acid bating treatment - Discontinuous processing**

| Products / conditions | m.u. | Paddle system | Overflow system | Jigger system |
|---|---|---|---|---|
| Dispersing emulsifying agent (mixture of non-ionic surfactants) | g/l | 1 - 2 | 1 - 2 | - |
| INVADINE DA (Ciba Speciality Chemicals S.p.A.) | | | | |
| Dispersing wetting agent (mixture of non-ionic surfactants) | g/l | - | - | 2 - 4 |
| ULTRAVON CN (Ciba Speciality Chemicals S.p.A.) | | | | |
| Acidifying agent | g/l | 1 - 3 | 1 - 3 | 2 - 4 |
| (derived from phosphoric acids with water-soluble polymers) | | | | |
| INVATEX SA (Ciba Speciality Chemicals S.p.A.) | | | | |
| Temperature | °C | 40 - 60 | 40 - 60 | 40 - 60 |
| Length of treatment | min | 30 -60 | 30 -60 | 45 - 90 |

**Acid bating treatment - Continuous cycle**

| **Products / conditions** | **m.u.** | **Cold storage** | **Continuous / short time** | **Continuous / long time** |
|---|---|---|---|---|
| **Dispersing wetting agent (mixture of non-ionic surfactants)** | g/l | 3 - 6 | 2 - 6 | 1 - 2 |
| **ULTRAVON CN (Ciba Speciality Chemicals S.p.A.)** | | | | |
| **Acidifying agent** | g/l | 4 - 8 | 6 - 12 | 2 - 4 |
| **(derived from phosphoric acids with water-soluble polymers)** | | | | |
| **INVATEX SA (Ciba Speciality Chemicals S.p.A.)** | | | | |
| Impregnation temperature | °C | 20 - 40 | 20 - 60 | - |
| Treatment temperature | °C | environmental temperature | 40 - 60 | 40 - 60 |
| Length of treatment | min | - | 0,5 - 2 | 1 - 3 |
| | hours | 2 - 6 | - | - |

The sequence of the processing steps can be considered, *per se,* analogous to the conventional direct printing process. Therefore, first of all there is a preparation step of the printing paste, ensuring the oxidative bleaching action according to the invention. A preferred preparation of the paste is expressed by the following recipe.

| **Chronological order** | **Products** | **Amount** (/kg) |
|---|---|---|
| 1 | **Purified water** | **as needed** |
| 2 | **Sodium hydroxide** (26 Be [Baumé degrees] solution) | 150 - 300 g |
| 3 | **Sequestering agent for heavy metals** (e.g. polyphosphonic acids in aqueous solution) MEPAL FA (Massimo Guarducci s.r.l.) | 3 - 5 g |
| 4 | **Wetting agent** (e.g. sodium alkane sulfonates with alkyldiols) INVADINE MR (Ciba Specialty Chemicals S.p.A.) | 10 - 15 g |
| 5 | **Stabilizing agent for hydrogen peroxide** (e.g. phosphoric derivatives containing ammina- diethylentriamine pentacetate-dipentasodium) H2O2 STABILIZING AGENT (Massimo Guarducci s.r.l.) | 20 - 30 g |

The presence of a complexing agent (sequestering agent) particularly important in case of presence of traces of heavy metals that, catalyzing the decomposition of the hydrogen peroxide, would cause depolymerizations of the cellulose with consequent weakening of the textile structures, up to the point of damaging the textile product as a result of the degradation of the cellulose caused by an unrestrained outburst of the oxidative action. The use of the wetting agent ensures a correct and homogeneous penetration of the printing paste in the textile substrate. The composition thus obtained is slowly agitated and then is added to with a thickening agent, according to the following specifications, so that the paste acquires the suitable thickness in view of the subsequent use.

| **Chronological order** | **products** | **Amount** (/kg) |
|---|---|---|
| 6 | **Thickening agent** (e.g. dispersion of acrylic copolymers in light mineral oil) - ALCOLPRINT DT-CS (Ciba Specialty Chemicals S.p.A.) | **55 - 65 g** |

The mixture is then quickly agitated until the desired viscosity is obtained. Finally, the hydrogen peroxide is added, possibly, after a further light agitation, along with the optical bleach, according to the following specifications.

| **Chronological order** | **products** | **Amount** (/kg) |
|---|---|---|
| 7 | **Hydrogen peroxide** (35%) | **150 - 300 g** |
| 8 | **Optical bleach** (if required) | **2 - 5 g** |
| | (e.g. derivative of stilbendisulfonic acid) | |
| | UVITEX BHT liquid or UVITEX CF liquid (Ciba Specialty Chemicals S.p.A.) | |

Then there follows the step of application of the printing paste on the textile fiber, an application that can take place, as stated, according to any one of the techniques already known, and therefore on conventional apparatuses. The printing speed shall vary, according to what can easily be optimized by an expert operator, according to the technique used and the results required. The penetration extent of the printing paste can also be adjusted according to the desired effect.

In the subsequent drying step, carried out as mentioned above, there develops the oxidative effect of the hydrogen peroxide, with the consequent localized degrading of the natural pigments and the formation of the print pattern. A steaming treatment can then take place; the steaming is not essential to obtain the desired print effect but can in any case be used to further develop the oxidative degradation effect. Such a treatment, if carried out in discontinuous apparatuses, can last 10÷20 minutes with saturated steam at a temperature of about 105°C. A final washing step with detergents has the purpose of eliminating the water-soluble oxidative demolition products and the residues of the printing paste. The washing can be carried out equivalently with discontinuous or continuous processes according to the apparatuses available. The washing temperatures and the other conditions are established, based upon common experience, according to the type of textile material and the type of apparatus used.

According to the invention, a printing process is thus disclosed that is able to achieve substantially new functional and aesthetic results, at least in relation to production methods of comparable simplicity and cost. As already stressed, the specifications of the example just described, although they should be considered advantageous in order to obtain an optimal result, must not be considered as a limitation.

In fact, variants and/or modifications can be brought to the printing process for obtaining surface designs on raw textile materials, and to the textile products thus obtained according to the present invention, without for this reason departing from the scope of protection of the invention itself as defined by the appended claims.

## Claims

1. A printing process to be used on a textile substrate made of natural and/or artificial cellulose fibers, alone or in combination with raw and/or dyed yarns of different composition, the process making use of a printing matrix on which there is formed a pattern to be reproduced, and comprising the step of directly applying on said substrate, by means of said printing matrix, a printing paste comprising an oxidative bleaching agent in an alkaline environment, **characterized in that** said textile substrate is a raw textile substrate, said oxidative bleaching agent is hydrogen peroxide, the alkalinity of said paste being controlled by means of a strong base, said oxidative agent and said strong base having, respectively, a concentration of between 150 and 300 g per kg of printing paste, said paste further comprising stabilizing agents and complexing agents for restraining the action of the oxidative agent and for preventing the start of catalytic reactions that could damage the fibers.

2. The process according to claim 1, wherein said strong base is sodium hydroxide.

3. The process according to claim 1 or 2, wherein said stabilizing and complexing agents comprise a stabilizing agent for hydrogen peroxide and a sequestering agent for heavy metals, in a concentration, respectively, between 20 and 30 g per kg of printing paste, and between 3 and 5 g per kg of printing paste.

4. The process according to any one of the previous claims, wherein said paste also comprises a wetting agent in a concentration of between 10 and 15 g per kg of paste.

5. The process according to any of the previous claims, wherein said paste also comprises an optical bleach in a concentration of between 2 and 5 g per kg of printing paste.

6. The process according to any of the previous claims, wherein said paste also comprises a thickening agent in a concentration of between 55 and 65 g per kg of paste.

7. The process according to any of the previous claims, wherein after the application of said printing paste said textile substrate is dried with hot air in a drying chamber with moderate ventilation at a temperature of between 65° and 110°C, for a time variable between 1 and 3 minutes.

8. The process according to claim 7, wherein after said drying step said textile substrate is left to rest folded in laps for 12 hours.

9. The process according to claim 7 or 8, wherein after said drying step said textile substrate is subjected to a steaming treatment and to a final washing step with detergents in order to eliminate the water-soluble oxidative demolition products and the residues of the printing paste.

10. The process according to any of the previous claims, wherein prior to the application of said printing paste, in order to eliminate the possible presence of traces of heavy metals, said textile substrate undergoes a bating and complexing pretreatment.

## Patentansprüche

1. Druckverfahren zur Verwendung auf einem Textilsubstrat, das besteht aus natürlichen und/oder künstlichen Zellulosefasern alleine oder in Kombination mit rohen oder gefärbten Garnen von verschiedener Zusammensetzung, welches Verfahren Gebrauch macht von einer Druckmatrix, auf welcher ein Muster ausgebildet ist, das zu reproduzieren ist, und den Schritt des direkten Aufbringens auf das Substrat mittels der Druckmatrix enthält, wobei eine Druckpaste ein oxidatives Bleichmittel in einer alkalischen Umgebung enthält, **dadurch gekennzeichnet, dass** das Textilsubstrat ein Rohtextilsubstrat ist, das oxidative Bleichmittel Wasserstoffperoxid ist, die Alkalinität der Paste mittels einer starken Base gesteuert wird, das oxidative Mittel und die starke Base jeweils eine Konzentration von zwischen 150 und 300 g pro kg der Druckpaste haben, die Paste ferner Stabilisierungsmittel und Komplexbildungsmittel zum Beschränken der Wirkung des oxidativen Mittels und zum Verhindern des Starts von katalytischen Reaktionen enthält, die die Fasern beschädigen könnten.

2. Verfahren nach Anspruch 1, wobei die starke Base Natriumhydroxid ist.

3. Verfahren nach Anspruch 1 oder 2, wobei die Stabilisierungs- und Komplexbildungsmittel ein Stabilisierungsmittel für Wasserstoffperoxid und einen Komplexbildner für Schwermetalle entsprechend in einer Konzentration von zwischen 20 und 30 g pro kg der Druckpaste und zwischen 3 und 5 g pro kg der Druckpaste enthalten.

4. Verfahren nach einem der vorhergehenden Ansprüche, wobei die Paste auch ein Befeuchtungsmittel in einer Konzentration von zwischen 10 und 15 g pro kg der Paste enthält.

5. Verfahren nach einem der vorhergehenden Ansprüche, wobei die Paste auch ein optisches Bleichmittel in einer Konzentration von zwischen 2 und 5 g pro kg der Druckpaste enthält.

6. Verfahren nach einem der vorhergehenden Ansprüche, wobei die Paste auch ein Eindickungsmittel in einer Konzentration von zwischen 55 und 65 g pro kg der Paste enthält.

7. Verfahren nach einem der vorhergehenden Ansprüche, wobei das Textilsubstrat nach dem Aufbringen der Druckpaste mit Heißluft in einer Trockenkammer mit moderater Ventilation bei einer Temperatur von zwischen 65° und 110°C für eine Zeit getrocknet wird, die zwischen 1 und 3 Minute(n) variabel ist.

8. Verfahren nach Anspruch 7, wobei das Textilsubstrat nach dem Trocknungsschritt 12 Stunden in Bahnen gefaltet zum Ruhen belassen wird.

9. Verfahren nach Anspruch 7 oder 8, wobei das Textilsubstrat nach dem Trocknungsschritt einen Dampfbehandlungs- und einem abschließenden Waschschritt mit Reinigungsmitteln unterzogen wird, um die wasserlöslichen oxidativen Schädigungsprodukte und die Reste der Druckpaste zu eliminieren.

10. Verfahren nach einem der vorhergehenden Ansprüche, wobei das Textilsubstrat vor dem Aufbringen der Druckpaste eine Beiz- und Komplexbildungsvorbehandlung durchmacht, um das mögliche Vorhandensein von Spuren von Schwermetallen zu elimieren.

## Revendications

1. Un procédé d'impression destiné à être utilisé sur un substrat textile réalisé avec des fibres de cellulose naturelles et/ou artificielles, seules ou en combinaison avec des fils bruts et/ou teints de composition différente, le procédé utilisant une matrice d'impression sur laquelle est formé un modèle à reproduire, et comprenant l'étape consistant à appliquer directement sur ledit substrat, au moyen de ladite matrice d'impression, une pâte d'impression comportant un agent de blanchiment oxydant dans un milieu alcalin, **caractérisé en ce que** ledit substrat textile est un substrat textile brut, ledit agent de blanchiment oxydant est du peroxyde d'hydrogène, l'alcalinité de ladite pâte étant ajustée au moyen d'une base forte, ledit agent oxydant et ladite base forte ayant, respectivement, une concentration comprise entre 150 et 300 g par kilogramme de pâte d'impression, ladite pâte comprenant en outre des agents stabilisants et des agents complexants pour restreindre l'action de l'agent oxydant et empêcher le démarrage de réactions catalytiques qui pourraient endommager les fibres.

2. Le procédé selon la revendication 1, où ladite base forte est de l'hydroxyde de sodium.

3. Le procédé selon l'une des revendications 1 et 2, où lesdits agents stabilisants et complexants comprennent un agent stabilisant pour le peroxyde d'hydrogène et un agent de séquestration pour métaux lourds, dans une concentration, respectivement, comprise entre 20 et 30 g par kilogramme de pâte d'impression, et comprise entre 3 et 5 g par kilogramme de pâte d'impression.

4. Le procédé selon l'une quelconque des revendications précédentes, où ladite pâte comprend également un agent mouillant dans une concentration comprise entre 10 et 15 g par kilogramme de pâte.

5. Le procédé selon l'une quelconque des revendications précédentes, où ladite pâte comprend en outre un agent de blanchiment optique dans une concentration comprise entre 2 et 5 g par kilogramme de pâte d'impression.

6. Le procédé selon l'une quelconque des revendications précédentes, où ladite pâte comprend en outre un agent épaississeur dans une concentration comprise entre 55 et 65 g par kilogramme de pâte.

7. Le procédé selon l'une quelconque des revendications précédentes, où, après l'application de ladite pâte d'impression, ledit substrat textile est séché avec de l'air chaud dans une chambre de séchage avec ventilation modérée à une température comprise entre 65°C et 110°C, pendant une durée variable comprise entre 1 et 3 minutes.

8. Le procédé selon la revendication 7, où, après ladite étape de séchage, ledit substrat textile est laissé plié au repos pendant un laps de temps de 12 heures.

9. Le procédé selon l'une des revendications 7 et 8, où, après l'étape de séchage, ledit substrat textile est soumis à un traitement à la vapeur et à une étape finale de lavage avec des détergents afin d'éliminer les produits de destruction oxydants hydrosolubles et les résidus de pâte d'impression.

10. Le procédé selon l'une quelconque des revendications précédentes, où, avant l'application de ladite pâte d'impression, afin d'éliminer la présence possible de traces de métaux lourds, ledit substrat textile subit un prétraitement de purification et complexant.
